

## UNITED STATES PATENT OFFICE

2,451,864

## EXPLOSIVES

Daniel P. O'Brien, Stamford, Conn.

No Drawing. Application May 15, 1945,  
Serial No. 593,971

1 Claim. (Cl. 52—15)

**1**

The invention here disclosed relates to explosives.

Objects of the invention are to provide explosives for use in bombs and the like which will have great disruptive force, be instantaneous in action and which while normally inert and inactive, may be set off or detonated by contact with water.

Other objects are to combine in an explosive the high temperature burning effects desirable in incendiary and demolition bombs and to accomplish this and the first mentioned objects with materials which are available at reasonable cost and which can be safely handled, combined and transported.

Other objects of the invention and the novel features by which the purposes of the invention are attained will appear in the course of the following specification.

Basically the invention comprises the combining of a high temperature burning medium having the characteristics of magnesium (Mg) with a water sensitizing agent having the characteristics of calcium phosphide (Ca<sub>3</sub>P<sub>2</sub>) and usually with an activating agent having the characteristics of potassium perchlorate (KClO<sub>4</sub>).

These materials preferably are all in powder form. In instances where rapid combustion is not so important the magnesium may be in the form of chips, and similarly the calcium phosphide may be in small grains or particles larger than normal powder size.

The magnesium may be in either the chemically pure form or in one of the commercial states, in which it may contain small proportions of other metals such as zinc, aluminum, copper and manganese.

Without restricting choice of materials, a commercial grade of magnesium found suited to the purpose is composed of

|           |         |
|-----------|---------|
| Magnesium | 99.8335 |
| Zinc      | .05     |
| Aluminum  | .064    |
| Copper    | .021    |
| Manganese | .03     |

in powder form of a fineness to pass through a 200 mesh screen.

Similarly the commercial grades of calcium phosphide and potassium perchlorate in 200 mesh powder form are suitable to the purposes of the invention.

While proportions may vary considerably, for high power flash bombing the following proportions by weight have been employed:

55

|                                                     |        |   |
|-----------------------------------------------------|--------|---|
| Magnesium (Mg)                                      | ounces | 2 |
| Calcium Phosphide (Ca <sub>3</sub> P <sub>2</sub> ) | drams  | 2 |
| Potassium Perchlorate (KClO <sub>4</sub> )          | dram   | 1 |

**2**

These materials, in dry powder form, may be mixed in any usual or ordinary way, under proper precautions to keep them dry during all mixing and handling operations.

Preferably the mixture when complete is loaded at once into bomb casings and sealed to prevent access of moisture. The bomb casings or shells may be of any material and form to keep the mixture dry and strong enough to withstand transportation and forces of propulsion and the like.

These water-tight containers may be of a type to burst on contact and more or less spread the contents, such construction enabling placing of the material by gunfire or dropping from aircraft and subsequent ignition or detonation of the deposited explosive by bombardment with bursting water shells, or if the element of surprise is desired, the detonation may be left to be effected by rain or liquidation of moisture from the air.

What is claimed is:

An explosive containing magnesium, calcium phosphide and potassium perchlorate in substantially the proportions by weight of 32 parts magnesium, 2 parts calcium phosphide and 1 part potassium perchlorate.

DANIEL P. O'BRIEN.

## REFERENCES CITED

The following references are of record in the file of this patent:

## UNITED STATES PATENTS

| Number    | Name      | Date          |
|-----------|-----------|---------------|
| 841,172   | Nienstadt | Jan. 15, 1907 |
| 1,045,671 | Bureau    | Nov. 26, 1912 |
| 1,342,802 | Gerli     | June 8, 1920  |
| 1,351,078 | Walker    | Aug. 31, 1920 |
| 1,404,653 | Ross      | Jan. 24, 1922 |
| 2,095,302 | Woodford  | Oct. 12, 1937 |
| 2,410,801 | Audrieth  | Nov. 12, 1946 |

## FOREIGN PATENTS

| Number  | Country       | Date          |
|---------|---------------|---------------|
| 12,137  | Great Britain | 1895          |
| 124,796 | Great Britain | Apr. 10, 1919 |
| 460,323 | Germany       | May 24, 1928  |

## OTHER REFERENCES

Barnett, "Explosives," London, 1919, pages 176 and 177.